

[54] ALKYLATED METHYLENEDIANILINE TARS

[75] Inventor: Robert Archie Gardiner, Wilmington, Del.

[73] Assignee: E. I. du Pont de Nemours and Company, Wilmington, Del.

[22] Filed: Jan. 20, 1972

[21] Appl. No.: 219,526

[52] U.S. Cl. .... 252/50, 260/568

[51] Int. Cl. .... C10m 1/34

[58] Field of Search..... 260/568; 252/50

[56] References Cited

UNITED STATES PATENTS

|           |         |                    |          |
|-----------|---------|--------------------|----------|
| 3,320,209 | 5/1967  | Bremmer .....      | 260/568  |
| 3,577,476 | 5/1971  | Gurney et al. .... | 260/568  |
| 3,004,916 | 10/1961 | Ertelt.....        | 252/32.7 |

Primary Examiner—Werten F. W. Bellamy  
Attorney—Francis J. Crowley

[57] ABSTRACT

Alkylated methylenedianiline tars having the formula



wherein each R is independently a secondary 2-alkyl radical having from about three to about 10 carbon atoms and n is from about 0.7 to about 1.2.

5 Claims, No Drawings

## ALKYLATED METHYLENEDIANILINE TARS

## BACKGROUND OF THE INVENTION

## 1. Field of the Invention

This invention relates to compositions consisting essentially of alkylated aromatic polyamines and more particularly to alkylated methylenedianiline tars which are useful lubricant additives.

## 2. Description of the Prior Art

To meet the requirements of modern technology, lubricants are usually compounded with additives. A lubricant additive may be defined as a material which imparts a new and desired property not found in the original base lubricant or which property reinforces one or more desirable properties already possessed to some degree by the base lubricant. Additives designated as antioxidants, corrosion inhibitors, rust inhibitors, extreme pressure agents, anti-stain agents, anti-wear agents, viscosity index improvers, pour point depressants, detergents, dispersants and the like are well recognized in the art. Lubricant bases into which such additives are blended include not only those derived from petroleum sources but synthetic lubricants as well. Synthetic lubricant bases of such types as aliphatic esters, polyalkylene oxides, silicones and fluorine-containing materials, for example, are also improved by the addition thereto of selected lubricant additives.

Most often the environment in which a lubricant is used is such that the lubricant comes into contact with air and metals which may function as pro-oxidants, often at elevated temperatures. Under such conditions, the lubricant, whether it be mineral oil based or synthetic based, undergoes a series of oxidation reactions whereby the viscosity of the lubricant is increased and carbonaceous deposits and acidic by-products are formed. The increase in viscosity and the formation of carbonaceous deposits may lead to impairment of lubricating ability of the lubricant, and the formation of acidic by-products may lead to increased corrosion of the metal parts which are in contact with the lubricant. Antioxidants are, therefore, regarded among the more important additives used in lubricant compositions. Lubricants protected by antioxidants include lubricating oils, synthetic lubricants and grease compositions. Classes of organic compounds used in the art as antioxidants include sulfides, disulfides, sulfoxides, phosphites, amines, phenols, selenides and zinc dithiophosphates. Particular choice of an antioxidant of course depends upon the lubricant base employed and the intended use of the lubricant.

Amines, particularly aromatic amines, have been used extensively as antioxidants in lubricants because of their effectiveness and because they possess desirable auxiliary properties such as good solubility in lubricant bases, compatibility with other additives, and their ready availability. In general the aromatic amines useful as antioxidants are those wherein the amine nitrogens contain alkyl or aryl substituents as exemplified by N-phenyl-alphanaphthylamine, N-phenyl-beta-naphthylamine, tetramethyl-diamino-diphenylmethane and phenothiazine.

It is also, however, recognized in the art that in addition to being effective for the intended antioxidant purpose and satisfactory in other additive requirements, such as solubility, a lubricant additive must also be economical to produce in order to obtain commercial acceptance.

Cyba et al. in U.S. Pat. No. 3,011,976 disclose lubricant compositions containing 4,4'-di-(sec. alkyl)-4,4'-diamino-diphenylmethane and N,N,N',N'-tetra-(sec. alkyl)-4,4'-dimainodiphenylmethane wherein the above diphenylmethane derivatives are obtained by reductive alkylation of 4,4'-diaminodiphenylmethane. One of the advantages cited by the patentee is the low cost of the use of such inhibitors produced from 4,4'-diaminodiphenylmethane. The above-disclosed diphenylmethane derivatives are, however, not considered to be adequately effective antioxidants in all applications and the cost of producing such diphenylmethanes is not as low as might be desired.

15 Novel compositions comprising alkylated aromatic polyamines have now been discovered, which are effective lubricant antioxidants and which can be economically produced.

## SUMMARY OF THE INVENTION

20 This invention is directed to compositions consisting essentially of alkylated aromatic polyamines having the formula



25 30 35 wherein each R is independently a secondary 2-alkyl radical having from about three to about 10 carbon atoms and n is from about 0.07 to about 1.2. Also included within this invention are lubricants comprising a lubricant base and a stabilizing amount of one or more of these compositions.

## DESCRIPTION OF THE INVENTION

40 45 This invention relates to compositions useful as lubricant additives. These compositions consist essentially of alkylated aromatic polyamines of the formula



50 55 60 wherein R is a secondary 2-alkyl radical having from about three to about 10 carbon atoms and wherein n is from about 0.7 to about 1.2.

65 As is well known in the art, methylenedianilines are much desired commercial compositions because of the versatility of their uses, e.g., in the preparation of epoxy resins, polyamides, polyimides, polyureas and polyurethanes and specifically 4,4'-methylenedianiline is also used extensively as an intermediate in the preparation 4,4'-methylene-diphenyldiisocyanate which is used in preparation of polyurethane polymers and as an intermediate in the preparation of antioxidants. These methylenedianilines are usually prepared by reacting aniline with formaldehyde in the presence of a strong acid catalyst such as hydrochloric acid, sulfuric acid, perchloric acid, hydrobromic acid, boron trifluoride, tin

tetrachloride, phosphorus chloride, phosphorus oxychloride, thionyl chloride, aluminum chloride and the like. In this reaction various isomeric methylenedianilines may be produced, including the 4,4'-isomer, the 2,4'-isomer and the 2,2'-isomer. In the usual condensation the 4,4'-isomer is present to the extent of about 90 percent and the 2,4'-isomer is present to about 10 percent, there being very small amounts of 2,2'-isomer present. For certain applications of the methylenedianilines, such as their use in the preparation of polyisocyanates with lower tendency to crystallize, a higher proportion of 2,4'-isomer is desirable, and by careful control of the aniline to formaldehyde ratio and of the aniline to water ratio, isomeric mixtures containing up to 35 percent of the 2,4'-isomer can be prepared (see U.S. Pat. No. 3,277,173). The yield of methylenedianiline from the condensation of aniline with formaldehyde normally ranges from about 40 percent to about 85 percent depending upon the particular process conditions.

When higher conversions and higher yields of the methylenedianilines are sought by the usual procedures of changing reactant ratios or by extending the heating time, the amount of unusable by-product is also increased. For example, when the 4,4'-isomer of methylenedianiline having the formula



and the 2,4'-isomer having the formula



react further with another molecule of formaldehyde and another molecule of aniline, identical products having the formula



are obtained.

Further condensation of the triamine (I) above, with formaldehyde and aniline, will produce a tetra-amine having the formula



It is also possible that the 2,2'-isomer which is present in very small amounts may also react further with formaldehyde and aniline to form a triamine which may be designated as 2,2'-diamino-5'-(methylene-p-aminophenyl)-diphenylmethane, however, the amount of such triamine which may be present is so small that for all practical purposes, the triamine may be considered to be entirely that exemplified by (I).

The above described triamine (I) and tetra-amine (II) are formed not only during the condensation reaction process itself but also during distillation recovery of the methylenedianilines, and particularly when such distillations are carried out to recover the last possible amounts of methylenedianilines by either prolonged heating or heating at higher temperatures. Thus, since from about 40 to about 85 percent of the starting materials used in the distillation of methylene-dianiline go into the methylenedianiline itself, the remaining about 60 to about 15 percent of the starting materials can be said to go into the methylenedianiline tar residue. There being little practical utility for the above-described methylene-dianiline tar residues, often referred to as "tars," they are usually discarded and, since there are no ready means for their disposal, they are burned by costly and time-consuming means. It is clear, therefore, that if any useful products can be prepared from these presently discarded methylenedianiline tar residues, such tar residues will afford a very inexpensive source for the starting materials used in the preparation of such useful products.

It has now been discovered that by reductive alkylation of methylenedianiline tar residues with methyl ketones containing from about three to about 10 carbon atoms, compositions useful as lubricant additives are obtained and moreover it has been discovered that such alkylated methylenedianiline tars are more effective as lubricant antioxidants than the alkylated methylenedianilines themselves.

As discussed above, the methylenedianiline tar residues are primarily mixtures of aromatic polyamines, there being present some 4,4'-methylenedianiline, 2,4'-methylenedianiline, 2,2'-methylenedianiline, triamine exemplified by formula (I) and some tetra-amine exemplified by formula (II). The amount of methylenedianilines present in the tar will, of course, depend upon the efficiency of the methylenedianiline recovery process, but in most cases methylenedianilines make up less than about 10 weight percent, and usually about three to about five weight percent of the tar residues obtained. The major portion of the methylenedianiline tar residue is the triamine of formula (I). The tetra-amine (II) normally makes up less than about five weight percent of the tar residue, but this too can vary according to the condensation and recovery processes.

The composition of the methylenedianiline tar residue may be represented by the formula



With respect to the above formula (III) in that portion of the tar residue which is methylenedianiline,  $n$  in formula (III) is 0, in that portion of the residue which is triamine as in formula (I),  $n$  in formula (III) is 1, and

where the tar residue is a tetra-amine as in formula (II),  $n$  in formula (III) is 2. However, since the tar residue is normally a mixture, the composition can be best represented by some intermediate value of  $n$ . Thus in an illustrative example of a mixture, where the tar is composed of 10 percent by weight of methylenedianiline and 90 percent by weight of triamine of formula (I),  $n$  will have a value of 0.87. It should be noted that the weight percentages of triamine, tetra-amine and methylenedianiline set out above are typically found in the tar residue, but as stated, the percentages of each may be greater or less depending on the various considerations mentioned previously.

The table below shows the values for  $n$  for various typical and atypical combinations of aromatic amines in the tar. In the table, MDA refers to methylenedianiline, "triamine" refers to a compound as exemplified by formula (I) and "tetra-amine" refers to a compound as exemplified by formula (II). The given value for  $n$  is weighted average of the  $n$  values of the components of the mixture.

Table

## MIXTURES OF AROMATIC POLYAMINES

| Mixture     | Weight % | Mol. % | $n$  |
|-------------|----------|--------|------|
| 1. MDA      | 20       | 28.7   |      |
| triamine    | 80       | 71.3   | 0.71 |
| 2. MDA      | 15       | 21.3   |      |
| triamine    | 85       | 78.7   | .79  |
| 3. MDA      | 10       | 13.4   |      |
| triamine    | 90       | 86.6   | 0.87 |
| 4. MDA      | 5        | 7.7    |      |
| triamine    | 95       | 92.3   | 0.92 |
| 5. MDA      | 1        | 1.4    |      |
| triamine    | 99       | 98.6   | 0.99 |
| 6. MDA      | 10       | 7.6    |      |
| triamine    | 80       | 78.2   | 0.93 |
| 7. triamine | 10       | 14.2   |      |
| tetra-amine | 90       | 92.4   | 1.08 |
| 8. triamine | 10       | 7.6    |      |
| tetra-amine | 75       | 80     | 1.2  |
|             | 25       | 20     |      |

It has been found by analytical means, including gas chromatography and nuclear magnetic resonance spectroscopy, that a typical methylenedianiline tar residue contains less than 10 percent by weight of methylenedianiline, less than about 5 percent by weight of tetra-amine and that the majority of the tar is made up of tri-amine of formula (I). Thus in formula (III) for the methylenedianiline tar residue, a typical tar will have a value of  $n$  in the range of from about 0.85 to about 0.99. Tar residues having an  $n$  value of from about 0.7 to about 1.2 are however still economical to use since they do not contain as much expensive MDA as to appreciably increase their cost and they do not contain sufficient MDA and tetra-amine to reduce their overall effectiveness as starting materials for the production of the effective lubricant additives of this invention. These tars are therefore useful in the preparation of the additives of this invention.

The compositions of this invention are prepared by reductive alkylation of a methylenedianiline tar residue. This reductive alkylation is carried out by treating the tar residue in excess methyl ketones preferably having from about three to about 10 carbon atoms (e.g., solvent quantities) with hydrogen at 100°C. to 250°C. in the presence of a suitable catalyst system. Suitable catalysts include the usual hydrogenation catalysts such as platinum, palladium, cobalt or nickel, either as such or carried on a suitable support, such as carbon. The reaction system may also contain catalysts which are

known to promote condensation of carbonyl compounds with aromatic amines to form anils; such catalysts include zinc chloride, acetic acid, phosphoric acid, alkyl acid phosphates and the like. Under the usual reaction conditions the products obtained are mono-substituted amine derivatives, i.e., each of the amino nitrogen has only one secondary alkyl group attached thereon. Thus the product obtained upon reductive alkylation of the methylenedianiline tar residue may be represented by



wherein  $n$  is from about 0.7 to about 1.2

Since the ketones useful in forming the compositions of the invention are methyl ketones of three to 10 carbon atoms the alkyl group attached to the amino nitrogen of the resultant aromatic polyamines are secondary 2-alkyl groups which may be represented by the formula  $-\text{CH}(\text{CH}_3)-\text{R}^1$  wherein  $\text{R}^1$  is an alkyl group having from one to about eight carbon atoms. The useful ketones are therefore methyl alkyl ketones wherein the alkyl portions are methyl, ethyl, propyl, butyl, pentyl, hexyl, heptyl and octyl as well as the various isomeric forms of the latter six alkyl groups. Specific, but non-limiting examples thereof include acetone, 2-butanone, 2-pentanone, 4-methylbutane-2-one, 2-hexanone, 4-methylhexane-2-one, 2-heptanone, 5-methylhexane-2-one, 5,6-dimethylhexane-2-one, 5,5-dimethylhexane-2-one, 4,5-dimethylhexane-2-one, 4-ethyl-hexane-2-one, 5-ethylhexane-2-one, 2-nonenone, 6-methyloctane-2-one, 5,5-dimethylheptane-2-one, 4,5-dimethylheptane-2-one, 4,5,5-trimethylhexane-2-one, 5-ethylheptane-2-one, 4-ethylheptane-2-one, 2-decanone, 7,7-dimethyloctane-2-one, 6-ethyloctane-2-one, and the like. The preferred ketone is 5-methylhexane-2-one so the preferred R group in the alkylated methylene dianiline tar of formula (III) is -



As stated previously, the ketones used in the reductive alkylation are methyl ketones having preferably from about three to about 10 carbon atoms. When methyl ketones containing from about three to about six carbon atoms are used, the resultant alkylated methylenedianiline tar residues are not very soluble in liquid lubricant bases, however, these products are effective antioxidants in lubricant compositions such as greases wherein complete solubility in the lubricant base is not necessarily required. When high solubility in lubricant bases is desired, methyl ketones of from about six to about 10 carbon atoms are used in the reductive alkylation process. While methyl ketones containing more than 10 carbon atoms are useful in the preparation of the alkylated products of the invention, the sluggishness of the reductive alkylation process and the limited availability of such ketones make them less desirable than the methyl ketones of three to 10 carbon atoms. A mixture of methyl ketones may be used in the

reductive alkylation process such that the resultant alkylated methylenedianiline tar will have a mixture of secondary 2-alkyl groups; however for simplified operation it is more convenient to use a single methyl ketone.

In the reductive alkylation process the completion of the reaction is usually indicated by the cessation of hydrogen absorption. The alkylated products may also be analyzed for the completion of alkylation by conventional procedures such as by infrared spectroscopy. If the alkylated methylenedianiline tar is to be used as an antioxidant in grease compositions, it has been found that complete alkylation is not necessary whereas if the product is to be used in lubricating oils, complete alkylation is desirable to obtain the required solubility.

The alkylated methylenedianiline tar residues of this invention are effective antioxidants in grease compositions and in lubricating oils. Unexpectedly, the alkylated methylenedianiline tar residues of this invention, as represented by formula (IV),  $n = 0.7 - 1.2$ , are more effective as antioxidants in greases and in lubricating oil than alkylated methylenedianilines which contain the same secondary 2-alkyl groups (formula IV,  $n = 0$ ). This fact is clearly borne out by the examples which follow. The present invention, therefore, provides effective antioxidant compositions which are also very economical to produce since the starting materials for their production are methylene-dianiline tar residues which are ordinarily discarded at considerable expense.

The compositions of the invention can be blended with the lubricant bases in any of the conventional methods such as adding them to the lubricant base and mixing or adding the compositions as a solution in a suitable solvent followed by mixing and topping of the volatile solvent. In blending of the compositions of the invention into grease compositions, the invention compositions may be added to the lubricant bases or added along with the grease thickeners. It will be readily apparent to those skilled in the art that the alkylated methylenedianiline tar residues of the invention may be used in lubricant compositions together with other lubricant additives which are normally used.

The following examples are intended to be merely illustrative of the invention and not in limitation thereof. Unless otherwise indicated, all quantities are by weight.

#### EXAMPLE 1

This example illustrates the preparation of alkylated methylenedianiline tar residues. Tar residue obtained from the methylenedianiline manufacturing process was analyzed by vapor phase chromatography and found to contain about 10 percent by weight methylenedianiline



Nuclear magnetic resonance (NMR) analysis indicated that the major constituent of the tar was the triamine represented by the formula



- 10 Three hundred sixty Grams of the tar residue in 592 g. of methylisoamylketone was charged into a 2-liter autoclave. To this mixture in the autoclave was added 4 g. of 85 percent (A. R. Grade) phosphoric acid, 8 g. of tridecyl acid phosphate, 30 g. of a hydrogenation catalyst, i.e., 1 percent platinum metal on carbon ("Darco" G-60), and 20 g. of distilled water. The autoclave was pressurized with hydrogen (400-500 psig) and then heated with shaking to about 170°C. Hydrogenation was continued at 170°C. and 400-500 psig hydrogen pressure. A major portion of hydrogen absorption occurred during the first 5 to 7 hours and thereafter continued slowly for an additional 8 to 9 hours, after which the hydrogen absorption ceased. The total hydrogen pressure drop was around 1,200 psig. The autoclave charge was filtered hot and then topped at 150°C. and 10 mm. pressure for 3-5 hours. The product obtained (628 g.) was a viscous transparent red material which was highly soluble (75 percent solution being readily obtained) in solvent refined neutral oil (100 SUS/100°F.). NMR analysis of the product indicated that the product obtained was mono-substituted amine derivative wherein each amine-nitrogen had only one methylisoamylmethyl group attached thereon. This product is therefore represented by the formula
- 20
- 25
- 30
- 35



wherein R is methylisoamylmethyl and n is 0.87.

45 Using the same general operating procedure described above, additional alkylated methylenedianiline tar residues in this invention were obtained using acetone, methylethylketone, methylisobutyl ketone, methylpentyl ketone and methylhexyl ketone. However, when ethylamyl ketone (octane-3-one) was used, no absorption of hydrogen took place.

#### EXAMPLE 2

55 This example illustrates the antioxidant activities and the superiority of the alkylated methylene-dianiline tar residues of this invention over the corresponding alkylated methylenedianiline when used as additives in lubricating grease. The comparative test method was the Oxygen Bomb Test, i.e., ASTM D-942, wherein a sample of grease containing the antioxidant additive composition is heated in a bomb to 210°F. (99°C.) and the bomb is filled with oxygen at 110 psi (7.7 kg. per sq. cm.), the pressure is then observed and recorded at stated intervals. The degree of protection afforded by the anti-oxidant composition is compared in terms of number of hours required for the oxygen pressure to drop 25 psi. The grease utilized throughout the com-

60

65

parative test was multi-purpose lithium-calcium grease sold by the Esso Corp. The results are shown in Table I below. In this table, C<sub>3</sub>-sec. alkyl group is isopropyl, C<sub>7</sub>-sec. alkyl group is methylisoamylmethyl, MDA is 4,4'-methylenedianiline and MDA-TAR is methylene-

in a single container of the oil at 250°F. for 168 hours while agitating with oil with air, and then checking for the changes in the metals and the oil. The results are summarized in Table III below. The alkylated compounds are designated as in Example 2.

TABLE III.—CORROSION AND OXIDATION OF LIGHT OILS

**Test Conditions; 250° F. for 168 Hours**

| Antioxidant                            | Conc.,<br>wt.<br>percent | Viscosity (cs. at 100° F.) |       |                   | Acid number |       |        | Metal coupons wt. loss (g.) |    |    |       |      |
|----------------------------------------|--------------------------|----------------------------|-------|-------------------|-------------|-------|--------|-----------------------------|----|----|-------|------|
|                                        |                          | Before                     | After | Percent<br>change | Before      | After | Change | Cu                          | Mg | Al | Steel | Cd   |
| 1.----- Turbine oil (Sun Oil Co.)----- | 0                        | 32.6                       | 68.7  | 110.7             | 0.02        | 12.30 | 12.28  | 0.004                       | 0  | 0  | 0     | 0.21 |
| 2.----- Cr-sec. alkyl MDA-----         | 0.05                     | 32.6                       | 66.4  | 103.6             | 0.02        | 13.10 | 13.08  | 0.004                       | 0  | 0  | 0     | 0.04 |
| 3.----- Cr-sec. alkyl MDA-TAR-----     | 0.05                     | 32.7                       | 37.9  | 15.9              | 0.02        | 2.60  | 2.58   | 0.003                       | 0  | 0  | 0     | 0    |
| 4.----- do -----                       | 0.50                     | 32.9                       | 33.3  | 1.2               | 0.02        | 0.05  | 0.03   | 0                           | 0  | 0  | 0     | 0    |

dianiline tar containing about 10 percent by weight of methylenedianiline isomers.

TABLE I

#### Grease Bomb Oxidation Test (ASTM D-942)

| Antioxidant                           | Conc., Wt. % | Hours to 25 psi<br>Pressure Drop |
|---------------------------------------|--------------|----------------------------------|
| 1. Control grease                     | 0            | 47                               |
| 2. C <sub>9</sub> -sec. alkyl MDA     | 0.5          | 535                              |
| 3. C <sub>9</sub> -sec. alkyl MDA-TAR | 0.5          | 854                              |
| 4. C <sub>7</sub> -sec. alkyl MDA     | 0.5          | 682                              |
| 5. C <sub>7</sub> -sec. alkyl MDA-TAR | 0.375        | 483                              |

Since the methylenedianiline tar residue (MDA-TAR) used to prepare the above alkylated products may contain up to 10 percent by weight of methylenedianiline and thus the alkylated tar residue may contain up to 10 percent of alkylated methylenedianiline, the following grease bomb oxidation tests were carried out as above using the same antioxidants but at 0.04 weight percent level. The results are shown in Table II below.

TABLE II

### Grease Bomb Oxidation Test (ASTM D-942)

| Antioxidant                            | Conc., Wt. % | Hours to 25 psi<br>Pressure Drop |
|----------------------------------------|--------------|----------------------------------|
| 6. Control grease                      | 0            | 68                               |
| 7. C <sub>9</sub> -sec. alkyl MDA      | 0.04         | 58                               |
| 8. C <sub>9</sub> -sec. alkyl MDA-TAR  | 0.04         | 85                               |
| 9. C <sub>7</sub> -sec. alkyl MDA      | 0.04         | 54                               |
| 10. C <sub>7</sub> -sec. alkyl MDA-TAR | 0.04         | 101                              |

These results clearly show the superiority of the alkylated methylenedianiline tar residues as antioxidants in grease compositions over the corresponding alkylated methylenedianilines. The results summarized in Table II also clearly show that the oxidant activity of alkylated methylenedianiline tar is not due to the possible presence of a small amount of alkylated methylenedianiline since the alkylated methylenedianilines as shown in Table II, 7 and 9, show no antioxidant activity at a comparable concentration.

### EXAMPLE 3

This example illustrates the antioxidant activity of the alkylated methylenedianiline tar residues of this invention when they are used in light lubricating oils and also shows their superiority over corresponding alkylated methylenedianiline. The tests were carried out according to Federal Test Method Standard 791B Method 5308.6 for the measurement of corrosiveness and the oxidation stability of light oils. This test is used to determine the resistance to oxidation and the tendency to corrode various metals of highly refined light oils. The test involves immersing five different metals

These results show the superiority of an alkylated methylenedianiline tar of this invention over an alkylated methylenedianiline in light oil. As can be seen in Table III, the alkylated methylenedianiline at 0.05 weight percent level offered practically no protection to the oil (compare changes in 100°F. viscosity and the development in acidity) whereas the alkylated methylenedianiline tar at the same concentration provided good protection. Use of higher concentration (0.5 weight percent) of alkylated methylenedianiline tar offers excellent oxidation protection to the turbine oil.

The foregoing detailed description has been given for clarity of understanding only and no unnecessary limitations are to be understood therefrom. The invention is not limited to exact details shown and described for obvious modifications will occur to one skilled in the art.

The embodiments of the invention in which an exclusive property or privilege is claimed are defined as follows:

- 35 1. Compositions consisting essentially of alkylated aromatic polyamines having the formula



wherein each R is independently a secondary 2-alkyl radical having from about three to about 10 carbon atoms and n is from about 0.7 to about 1.2.

- 50 2. Compositions according to claim 1 wherein R is a 2-alkyl radical having the formula



wherein R' is an alkyl group having from one to about eight carbon atoms.

3. Compositions according to claim 2 wherein R is



4. Compositions according to claim 1 wherein  $n$  is from about 0.85 to about 0.99.

- 65 5. A lubricant comprising a lubricant base and a stabilizing amount of compositions consisting essentially of alkylated aromatic polyamines having the formula



wherein each R is independently a secondary 2-alkyl radical having from about three to about 10 carbon atoms and n is from about 0.7 to about 1.2.

5

\* \* \* \* \*

10

15

20

25

30

35

40

45

50

55

60

65